

Sept. 29, 1925.

1,555,237

A. V. CARLSSON

CASTING INGOTS

Filed Aug. 25, 1921

Fig. 1.



Fig. 2.



Fig. 3.  $b_2$



Inventor  
A. V. Carlsson,

By Market Clerk  
Atty's.

## UNITED STATES PATENT OFFICE.

ADOLF VERNER CARLSSON, OF KOLNSVA, SWEDEN.

## CASTING INGOTS.

Application filed August 25, 1921. Serial No. 495,151.

(GRANTED UNDER THE PROVISIONS OF THE ACT OF MARCH 3, 1921, 41 STAT. L., 1313.)

*To all whom it may concern:*

Be it known that I, ADOLF VERNER CARLSSON, a subject of the King of Sweden, residing at Kolsva, Sweden, have invented 5 certain new and useful Improvements in or Relating to Casting Ingots (for which I have filed application in Sweden, Nov. 14, 1918, Patent No. 49,093, of April 21, 1921; England, November 13, 1919, Patent No. 10 135,207; Norway, November 25, 1919; Denmark, Nov. 12, 1919; and Germany, November 27, 1919), of which the following is a specification.

When casting steel in a sand mould or an 15 ingot mould, the composition and the temperature of the steel being such as to produce steel without blisters, a more or less deep funnel-shaped depression called the pipe will be formed in the upper portion of 20 the ingot. The longer the upper portion of the ingot can be kept in a fluid state, the better can blow-holes which may appear in the ingot, be filled with molten metal from portions higher up and the smaller will be 25 the pipe. To retard solidification in the upper portion, a number of different methods are employed such as:—

(a) Building up or ramming the upper portion of ingot mould with fireproof material.

(b) Pouring slag on the fused steel.

(c) Supplying heat to the upper surface of the steel by ignited charcoal, thermite, or by electric heating.

35 Moreover, it is well known that carbon in some form or other is used in combination with moulding material, thus for instance cores are filled with coke for venting said cores, compressed carbon is introduced

40 in the walls of moulds for carburization or hardening of the steel cast, cores are made of fireclay or sand mixed with powdered graphite, and hollow cores have been made of a mixture, one element of which is combustible material for the purpose of obtaining combustion when the metal is cast.

45 By the present invention heat is transferred to the upper part of the ingot mould thus retarding the solidification of the dead head at this part and allowing molten metal to flow down and prevent formation of pipe underneath dead heads.

The present invention consists principally in ramming the walls of the feeding head

or the dead head with a material evolving 55 heat under the influence of the cast metal and transferring heat to the dead head, said heat-evolving material being mixed with strengthening ingredients and, if desired, acting as a heat insulator and protected 60 against contact with the metal. Materials of this character are charcoal, coal and coke in the form of powdered or crushed to grains of suitable size and preferably mixed with clay and other ingredients required for obtaining the necessary rigidity of the mould when ramming it and drying the material. The walls of the dead head or feeding head are preferably coated with blacking, or they are given a thin lining of some fireproof 70 paste to prevent the molten metal from coming into contact with the charcoal and thereby absorbing carbon.

Preferably the feeding head made in this way is only partly filled with metal, when 75 casting. Above this body of metal there is then deposited a layer of a material, such as charcoal, which will evolve heat under the influence of the cast metal, an insulating stratum being preferably arranged in 80 known manner between the molten metal and the charcoal, in order to prevent absorption of carbon. In accordance with this invention, the said insulating stratum may consist of molten slag or fused metal, the 85 specific gravity of which is lower than that of the metal thereunder. The slag cover can, however, be omitted if the charcoal is applied only after the solidification of the upper surface of the metal, an insulating 90 stratum preventing absorption of carbon having thus been formed already through the said solidifying action of the metal.

Any heat-evolving material can be advantageously used, provided that the heat 95 from the fused metal causes combustion of same, or gives rise to a reaction whereby heat is evolved.

To illustrate the method, Figures 1 and 2 of the accompanying drawing show a runner opening or feeding head in vertical section, the said figures being illustrative of the novel features according to the invention, whereas

Figure 3 is a vertical section of a runner 105 opening as heretofore known.

In Figure 1, *a* is the fused metal filling up the mold to the level *b*—*b*. *c* is the sand

mold, and  $d$  is the dead head in which is rammed the heat-evolving and heat-insulating material  $e$  containing coal.  $f$  is a thin stratum preventing the body from coming into direct contact with the molten metal.  $g$  is heat-evolving material such as charcoal, and  $h$  is an insulating heated layer serving the same purpose as the stratum  $f$ . The layer on the top surface may consist of a solidified stratum of the metal  $a$  itself, the same having the position  $h_1$  shown by dotted lines.

Figure 2 shows the appearance of the metal  $a$  after solidification. The top surface has then sunk down evenly and assumes the position indicated by the broken line  $b_1$   $b_1$   $b_1$ . The section shows a perfectly dense material, and the steel practically holds as much carbon in the upper part as in the lower part of the ingot.

Figure 3 shows the same metal cast in an ordinary sand mold, the ingot being shown immediately after casting and solidification of same. In the fused state the metal fills the mold up to the level  $b_2$   $b_2$ , that is to say as high up as in Figure 1. This surface remains unchanged, that is to say the metal solidifies at the surface and remains at this level. The solidification also begins immediately from the walls of the feeding head and, in fact, from the walls of the entire mould, while the central portions of the metal are still molten. The solidification is continued from the surface inwardly, the metal shrinks, and the metal from the middle of the upper part sinks down, but when the metal at the top surface and at the walls of the feeding head has solidified, the metal cannot sink any further, this resulting in the formation of a hollow-space or pipe, having an approximate form and extension as shown at  $k$  in Figure 3.

The present invention is particularly applicable to steel castings. The dead heads in steel castings serve the same purpose as the dead head (taken in the meaning of the metal cast in the feeding head) of ingots made with feeding heads, or the upper portion of ingots made without a feeding head, that is to say they are employed as reservoirs for fused metal, introduced to fill hollow spaces appearing in the ingot during the solidification of same. To this end the size of the dead heads must be considerable, as only a small portion of the metal cast into the dead head is effective, filling the space cavities in the ingot, the greater part of the metal solidifying in the dead head around the walls. It is the cooling from the walls that has to be prevented, this being brought about by making the wall so as to evolve heat, when coming in contact with the metal. The fused metal coming in contact with the walls, the carbon is caused to glow and evolves heat, thereby counteract-

ing the radiation of heat from the metal and thus retarding the solidification. The ineffective part of the dead heads, which is rammed in the known manner and which can be used only as scrap iron, ordinarily amounts to more than half the weight of the finished steel casting, counted on the average of the whole production, the waste of material thus being considerable.

Large dead heads have a disadvantageous influence also on the quality of the casting, that is to say, in so far as they are acting to the formation of cracks due to shrinking as well as to blow holes in the material.

The cracks are formed when on the cooling of the metal and the shrinking of it caused thereby, the strength of the material is insufficient to resist the stresses arising by the mold preventing the free shrinking of the metal. Blow holes will arise in that part of the section, which is the last to solidify, when on the solidifying of the metal the volume is reduced and the space cavity forming cannot be filled with fused metal from other parts. High temperature and a slow solidification and cooling act to produce cracks and blow holes. The solidification is accelerated, when the heat of the metal is quickly led off by the wall of the mould and thus a low temperature of the mould wall is an advantage, conditions otherwise remaining the same.

The steel having been cast in the mould, it will be cooled by the cold walls of the mould, but the more metal passing through the mould, the more the walls of the mould will be heated, and the less will be the cooling of the steel, the more the temperature of the metal approaches the maximum, that is to say the temperature of the metal running from the ladle.

Steel castings being mostly cast by bottom gate, that is to say, by introducing the steel into the bottom part of the mold, the steel filling the mould from the bottom upwards, the material, which fills the feeding heads, first passes through the mould. Even if the pouring is interrupted, such procedure being also practised, when the metal reaches the feeding head, that is to say when the metal has just filled the mould proper, and the steel is then poured into the feeding heads in order to obtain hotter metal in the latter, the pouring of the metal evidently is carried out first into one and then into another feeding head, but as the feeding heads communicate through the mould, the steel obviously passes through the latter. Thus, the larger the volume of the feeding heads relatively to the mould, the more metal will pass through the mould, the less will be the cooling of the metal and the greater the heating of the walls of the mould, the slower does the solidification take place and the greater will be the tendency of cracking

and sucking. By ramming the feeding heads in the manner set forth with a material evolving heat by the influence of the metal, the feeding heads are rendered more 5 efficient and thus their volume can be reduced so as to counteract crackings and blow holes.

It is to be understood that the heat-evolving material, such as charcoal, added to the 10 metal, must not come into contact with fused metal, this being prevented according to the present method by applying either molten slag or fused metal of a lower specific gravity than the metal itself, in which 15 case the melting temperature of the slag or the applied metal is utilized, or, in known manner, there may be added a material such as borax, which affords an insulating stratum and which is caused to glow or melt 20 by the metal, in which case, however, part of the heat is taken from the metal. It is also possible to mix the heat-evolving material, such as carbon in some form or other, with suitable substances giving a slag of high 25 fusibility, for instance lime and infusorial earth or powdered glass, and to cover the surface with this mixture thus producing a molten, an insulating stratum between the carbon and the iron. It is, moreover, possible 30 to let the top surface of the metal solidify and immediately thereafter apply the charcoal. The point is to get the charcoal burning so as to evolve heat to the metal and simultaneously to prevent the 35 charcoal from coming in direct contact with the fused metal.

The present method is particularly ap-

plicable to steel, but may obviously be used also in casting iron and other metals.

What I claim as new and desire to secure 40 by Letters Patent of the United States is:—

1. A method of preventing the formation of "pipe" in ingots and castings and of reducing the dead heads thereof, and thus of counteracting cracks and blow holes in 45 castings, consisting in ramming the walls of the feeding head or the dead head with a material, such as coal breeze, evolving heat under the influence of the cast metal and transferring heat to the dead head, said 50 heat-evolving material being mixed with strengthening ingredients and acting as a heat insulator.

2. A method according to claim 1, in which the heat-evolving material is mixed 55 with clay or the like for the purpose specified.

3. In a method according to claim 1 placing an insulating stratum between the fused metal and the heat-evolving material in 60 order to prevent absorption of the latter.

4. In a method according to claim 1, allowing the top surface of the metal to solidify and thus form an insulating stratum above 65 which a layer of heating material, as charcoal or the like, is placed and ignited in known manner.

5. A mould having the walls thereof rammed with a material, such as charcoal-breeze which is heat-insulating and heat-evolving under the influence of the metal 70 for the purposes specified.

In testimony whereof I affix my signature.

ADOLF VERNER CARLSSON.